

Sept. 4, 1973

SEIICHI TAGUCHI ET AL

3,756,817

METHOD FOR CORRECTION OF COLOR IMAGES

Filed Sept. 9, 1971

FIG.1



FIG.2



1

3,756,817

**METHOD FOR CORRECTION OF COLOR IMAGES**  
Seiichi Taguchi, Keishiro Kido, Akinori Kimura, Takeshi Tomatsu, and Eiichi Mizuki, Asaka, Japan, assignors to Fuji Photo Film Co., Ltd., Kanagawa, Japan  
Filed Sept. 9, 1971, Ser. No. 178,971  
Claims priority, application Japan, Sept. 9, 1970,  
45/79,022  
Int. Cl. G03f 3/00, 3/04; G03c 5/44  
U.S. Cl. 96—12 16 Claims

## ABSTRACT OF THE DISCLOSURE

Color images produced by dyeing gelatin reliefs containing silver are color corrected by rehalogenating the gelatin relief and then subjecting it to a tanning development. This treatment controls the dye-absorbing ability of the gelatin relief.

## BACKGROUND OF THE INVENTION

### Field of the invention

The present invention relates generally to a method for the correction of color images and more particularly it is concerned with a novel process for correcting colors, gradations, or optical densities in the formation of color images by a dye transfer process.

### Description of the prior art

A dye transfer process has hitherto been known and is fundamentally composed of the following four steps: (1) engraving, (2) dyeing, (3) rinsing, and (4) dye transferring.

The engraving step is also called a matrix making step and generally means such a step that a color negative film is printed on panchromatic matrix films (the main constituent of the film is composed of a dispersion of silver halide and pigment in unhardened gelatin) by a three-color separation system. The films are then subjected to tanning development and fixing so that a relief is formed on the films. In the tanning development, the areas of the film exposed to light are blackened and the unhardened gelatin of the film is hardened in proportion to the blackening. The fixing of the film is conducted by using a fixing solution containing sodium thiosulfate as the main component and containing no hardening agent. The formation of relief is conducted by removing the areas of the film with hot water that have not been exposed to light, i.e., those areas where the gelatin has not been hardened.

The dyeing step is a step of dyeing the gelatin of the matrix prepared in Step 1. In general, in this step each of a set of three matrices separated by lights of blue, green, and red is dyed in the corresponding color, i.e., dyed by a dyeing solution of yellow, magenta, or cyan dye respectively.

In the rinsing step, the excessive dyeing solution having no relation to the image, which has attached on the surface of the matrix thus dyed is removed.

In the dye transfer step, a dye-receiving paper having a mordanted gelatin layer is closely brought into contact with the gelatin layer of the matrix prepared above, whereby the dye in the matrix is transferred onto the dye-receiving paper. By transferring the dye images of yellow, magenta, and cyan successively onto a same image-receiving paper while strictly conforming the positions of the images, a natural color positive image can be obtained.

For adjusting the color, gradation, or density of the color image in the case of making the color image by the

2

dye transfer process as mentioned above, the following six methods have hitherto been known:

Method 1: By adjusting the pH of the dyeing solution, the amount of the dye to be adsorbed on the matrix is adjusted.

Method 2: By adjusting the pH of the rinsing solution, the amount of removal of the dye adsorbed on the matrix is adjusted.

Method 3: If the amount to be corrected is large, the exposure of the panchromatic matrix film is conducted again.

Method 4: If it is necessary to correct a part of the image, the film is exposed again while covering partially other areas than the part to be corrected.

Method 5: The undyed matrix is treated with an aqueous potassium permanganate solution to modify locally the gelatin layer, whereby the power of the gelatin layer absorbing the dye is weakened to the necessary extent.

Method 6: A necessary amount of the dye is removed from the matrix dyed by means of a brush containing a washing solution having a pH value higher than that of the dyeing solution.

These conventional methods have the following demerits respectively:

Method 1: It is difficult to maintain grey balance.

Method 2: The maintenance of grey balance is difficult and uneven dyeing is apt to occur.

Method 3: This method requires additional materials and difficulties are encountered.

Method 4: This method requires additional troubles and period of time.

Method 5: The control for the treatment is difficult and uneven dyeing is apt to occur.

Method 6: The control for the treatment is difficult and the treatment requires great skill. In case a large number of duplicates are to be produced, each duplicate must be retouched by hand, which reduces the reproducibility.

## SUMMARY OF THE INVENTION

It is the object of this invention to provide a method for correcting color images without the accompanying demerits as mentioned above.

The inventors have discovered that when a matrix having a relief is processed with a rehalogenation bath and then again developed with a tanning developing solution, the gelatin in the matrix is greatly modified and the absorbing ability of the gelatin for dye is remarkably disturbed. By applying such a phenomenon as discovered by the inventors, the method of this invention for correcting the color images by a dye transfer process has been accomplished. Thus, the invention is a method for correcting color images which comprises, in case of making the color images by a dye transfer process, rehalogenating the gelatin relief containing silver and then subjecting the gelatin relief to a tanning development to control the dye-absorbing ability of the gelatin relief.

## BRIEF DESCRIPTION OF THE DRAWING

An embodiment of the process of this invention is explained by referring to the accompanying drawings in which

FIG. 1 shows three views each illustrating the method of this invention and FIG. 2 is a graph showing the merits obtained by the method of this invention.

## DESCRIPTION OF THE PREFERRED EMBODIMENTS

FIG. 1(a) is a cross sectional view of a sheet having a gelatin relief image 11 on a support 10 prepared by a tanning development, fixing and wash-off process. Silver has been formed in the gelatin relief. The sheet is processed in a bleaching solution for silver, whereby the silver

present in the relief is rehalogenated as shown in FIG. 1(b). Thereafter, the sheet is developed again in a tanning developing solution whereby the gelatin of the relief image is modified and has a lowered adsorptive ability for dye as shown in FIG. 1(c). By conducting the dyeing and dye transferring by using the matrices thus prepared according to the ordinary manner, a corrected color image is obtained.

By repeating the silver bleaching-tanning developing steps as mentioned above, the color image can be corrected to a desired extent. This is shown in FIG. 2 in which the optical density is plotted to the logarithm of the exposure amount (abscissa). In FIG. 2 the curve 1 is the characteristic curve in the case where a matrix having a relief prepared by an ordinary manner is dyed and dye-

tion. For instance, a tanning developing solution containing pyrogallol, catechol, etc., may be emp'oyed.

The correction process of this invention may be applied to either the whole image or a part of the image. In case 5 of correcting the whole color image, the matrix is rehalogenated by, preferably, immersing the whole matrix in the rehalogenating solution. Also, in case of correcting the color image locally, the rehalogenating solution may be applied to the necessary part of the color image 10 by using a brush or the like. Such an operation can be conducted by persons skilled in the art without difficulty. The matrix corrected desirably by the process of this invention can be used as in the case of a usual matrix. Examples of dyeing step and dye transferring step are 15 shown below.

TABLE I

|                                      |                                    |                                                   |                                    |
|--------------------------------------|------------------------------------|---------------------------------------------------|------------------------------------|
| Dyeing solution.....                 | Cyan.....                          | Magenta.....                                      | Yellow.....                        |
| Dye.....                             | Anthraquinone Blue AB (C.I. 63010) | Anthraquinone Rubinol R concentrated (C.I. 68215) | Tartrazine (C.I. 19140) 2.0 grams. |
|                                      | 1.5 grams.                         | 3.0 grams.                                        |                                    |
| Sodium hydrogenphosphate.....        | 7.5 grams.....                     | 12.5 grams.....                                   | 20.0 grams.                        |
| Borax.....                           | 7.0 grams.....                     | 5.0 grams.....                                    | 2.2 grams.                         |
| Formalin (37% aqueous solution)..... | 10 milliliters.....                | 10 milliliters.....                               | 1 liter.                           |
| Water to make.....                   | 1 liter.....                       | 1 liter.....                                      | 5 minutes.                         |
| Dyeing time at 20° C.....            | 5 minutes.....                     | do.....                                           | Do.                                |
| Dye transferring time at 20° C.....  | do.....                            |                                                   |                                    |

transferred. Also, each of the cuves 2, 3 and 4 is the characteristic curve of the case where a matrix having a relief is subjected, once, twice or thrice respectively, to the bleach-tanning development steps of this invention and then dyed and dye transferred. From the results shown in FIG. 2 it will be understood that the density and gradation of color images can be controlled by repeatedly applying the process of this invention.

The gelatin relief used in the process of this invention may be composed of gelatin alone or may contain other high molecular weight material. For instance, gelatin containing about 0 to 10% by weight of polyvinyl alcohol or polyvinyl pyrrolidone may be used. The weight ratio of silver to gelatin in the gelatin relief is 1 to 3. Thus, the term "gelatin relief" means the relief made of such gelatin or gelatin composition.

The silver bleaching solution or rehalogenation solution used in this invention is an ordinary silver dye bleaching solution used in general photographic processings. That is to say, the silver bleaching solution contains an oxidizing agent and a halide. The typical example of the rehalogenating solution has, for instance, the following composition.

#### Rehalogenating Solution 1:

|                              |         |    |
|------------------------------|---------|----|
| Potassium ferrocyanide ..... | g..     | 30 |
| Potassium bromide .....      | g..     | 10 |
| Water .....                  | liter.. | 1  |

Rehalogenating Solution 2: (a mixture of the following Solution A, Solution B and water in a ratio of 1:1:5 is used).

#### Solution A:

|                                  |         |    |
|----------------------------------|---------|----|
| Potassium bichromate .....       | g..     | 20 |
| Concentrated sulfuric acid ..... | ml..    | 14 |
| Water .....                      | liter.. | 1  |

#### Solution B:

|                       |         |    |
|-----------------------|---------|----|
| Sodium chloride ..... | g..     | 45 |
| Water .....           | liter.. | 1  |

Rehalogenating Solution 3: (a mixture of the following Solution A and Solution B in a ratio of 1:1 is used).

#### Solution A:

|                      |         |     |
|----------------------|---------|-----|
| Copper sulfate ..... | g..     | 160 |
| Water .....          | liter.. | 1   |

#### Solution B:

|                            |         |     |
|----------------------------|---------|-----|
| Potassium bromide .....    | g..     | 100 |
| Potassium bichromate ..... | g..     | 2   |
| Water .....                | liter.. | 1   |

The tanning developing solution used in the process of this invention may be an ordinary tanning developing solu-

tion. For instance, a tanning developing solution containing pyrogallol, catechol, etc., may be emp'oyed.

The correction process of this invention may be applied to either the whole image or a part of the image. In case 5 of correcting the whole color image, the matrix is rehalogenated by, preferably, immersing the whole matrix in the rehalogenating solution. Also, in case of correcting the color image locally, the rehalogenating solution may be applied to the necessary part of the color image 10 by using a brush or the like. Such an operation can be conducted by persons skilled in the art without difficulty. The matrix corrected desirably by the process of this invention can be used as in the case of a usual matrix. Examples of dyeing step and dye transferring step are 15 shown below.

According to the process of this invention, the aforesaid six demerits common to the conventional method shown before can be remarkably improved, that is to say, the following demerits:

- 30 (1) the maintenance of grey balance is difficult,  
 (2) they require much skill, materials, and time,  
 (3) the color image is apt to become uneven.

The main reason is in the point that the color image 35 can be corrected in proportion to the amount of silver present in the matrix corresponding to the amount of exposure. It is also an important feature for practical purposes that the operation of this process can be carried out in a light room without the necessity of a dark room as in methods 3 and 4.

Also, by the process of this invention the color image 40 of the matrix is corrected permanently and hence the process of this invention is particularly effectively applied to the case of reproducing a large number of duplicates. Furthermore, it is also a feature of this invention that 45 there occurs no remarkable unnatural peripheral coloring which is apt to occur at the case of partial printing while covering other portions than the necessary areas.

Now, the invention is described more in detail by the following examples.

#### EXAMPLE 1

This example is the case of applying the method of this invention to the control of gradation.

A commercially available matrix film was wedge-exposed to red light and subjected to tanning development, fixing and relief making according to conventional methods. The matrix thus processed was dyed according to the treatment by the cyan dyeing solution shown in Table 1 described above and then subjected to washing and dye transferring to obtain the wedge image of cyan color. The contrast of the image was 1.36. Then, the matrix was immersed for 1 minute at 20° C. in the rehalogenating Solution 1 mentioned above and after washing with water, the matrix was developed for 2 minutes at 20° C. in the tanning developing solution having the following composition:

|                         | G.  |
|-------------------------|-----|
| Pyrogallol .....        | 8   |
| Sodium hydroxide .....  | 3   |
| Ammonium chloride ..... | 1.5 |
| Potassium bromide ..... | 1.5 |
| Citric acid .....       | 0.2 |
| Water, 1 liter.         |     |

After water washing, the matrix was dyed as mentioned above, washed, and then subjected to dye transfer step to

obtain the wedge image of cyan color. The contrast of the image was 1.05.

Similarly, the processings of the silver bleaching step and the tanning developing step were conducted repeatedly. The contrast of the wedge image of cyan color when the processings were conducted twice was 0.84 and that of the wedge image when the processings were conducted thrice was 0.75.

By applying the process as above to general color originals to control the contrast of the color image good reproductions can be obtained.

### EXAMPLE 2

This example is the case of applying the method of this invention to color correction.

After conducting similar procedures to the above example using a color original having colors of the skin and blue sky, only the part of blue sky image of the magenta matrix obtained by green separation was treated with the rehalogenation Solution 2 mentioned above by means of a brush for removing excess magenta dye at the blue sky image portion and then, after water washing, was developed for 2 minutes at 20° C. in the tanning developing solution having the following composition:

|                   | G.  |
|-------------------|-----|
| Catechol          | 7   |
| Sodium hydroxide  | 3   |
| Ammonium chloride | 1.5 |
| Potassium bromide | 1.5 |
| Citric acid       | 0.2 |
| Water, 1 liter.   |     |

By conducting the reproduction of color images by using the matrix thus obtained, a preferred color image having the color of a less reddish blue sky was obtained. When the color of the skin was maintained at a desirable color, the green optical density of the portion of the blue sky image was improved to 0.5 from a density of 0.3 before the correction treatment.

What we claim is:

1. In a method for forming a color image using the dye transfer process which comprises preparing at least one gelatin-relief-image-containing matrix from a silver halide light-sensitive gelatin containing element, applying a dye to said gelatin-relief-image-containing matrix, and transferring said dye from said gelatin-relief-image-containing matrix to a receptor surface to form said color image, the improvement which comprises, prior to said applying of said dye, correcting said color image by rehalogenating a portion of or all of said gelatin-relief-image-containing matrix, and then subjecting said rehalogenated gelatin-relief-image-containing matrix to a tanning development whereby the dye adsorbing ability of said gelatin-relief-image-containing matrix is controlled.

2. A method for forming a color image as claimed in claim 1, wherein the weight ratio of silver to gelatin in the gelatin-relief-image-containing matrix is 1 to 3.

3. A method for forming a color image as claimed in claim 1, wherein said gelatin-relief-image-containing matrix is gelatin alone, gelatin and polyvinyl alcohol or gelatin and polyvinyl pyrrolidone.

4. A method for forming a color image as claimed in claim 3, wherein said gelatin-relief-image-containing matrix contains about 0 to 10% by weight of polyvinyl alcohol.

5. A method for forming a color image as claimed in claim 3, wherein said gelatin-relief-image-containing matrix contains about 0 to 10% by weight of polyvinyl pyrrolidone.

6. A method for forming a color image as claimed in claim 1, wherein said rehalogenation solution contains an oxidizing agent and a halide.

7. A method for forming a color image as claimed in claim 6, wherein said oxidizing agent is potassium ferrocyanide, potassium bichromate, concentrated sulfuric acid or copper sulfate.

5 8. A method for forming a color image as claimed in claim 6, wherein said halide is potassium bromide or sodium bromide.

9 A method for forming a color image as claimed in claim 1, wherein said tanning development solution contains pyrogallol or catechol.

10 10. A method for forming a color image as claimed in claim 1, wherein said method comprises preparing one said gelatin-relief-image-containing matrix, whereby a mono-color image is formed.

15 11. A method for forming a color image as claimed in claim 1, wherein said method comprises preparing multiple gelatin-relief-image-containing matrices, applying a different dye to each of said gelatin-relief-image-containing matrices, and transferring each of said dyes from each of said gelatin-relief-image-containing matrices to a receptor surface, whereby a multicolor image is formed.

12. A method for forming a color image as claimed in claim 1, wherein said method comprises preparing multiple complementary gelatin-relief-image-containing matrices, applying a different dye to each of said gelatin-relief-image-containing matrices, and transferring each of said dyes from each of said gelatin-relief-image-containing matrices to a receptor surface, to form a multicolor image.

25 13. A method for forming a color image as claimed in claim 1, wherein said method comprises preparing complementary gelatin-relief-image-containing matrices, applying a different but complementary dye to each of said gelatin-relief-image-containing matrices, and sequentially and superimposedly transferring each of said dyes from each of said gelatin-relief-image-containing matrices to a receptor surface, whereby a multicolor image is formed.

30 14. A method for forming a color image as claimed in claim 1, wherein said method comprises preparing three complementary gelatin-relief-image-containing matrices, applying a different but complementary dye to each of said gelatin-relief-image-containing matrices, and sequentially and superimposedly transferring each of said dyes from each of said gelatin-relief-image-containing matrices to a receptor surface, to form a multicolored image.

40 15. A method for forming a color image as claimed in claim 14, wherein one of said gelatin-relief-image-containing matrices corresponds to the yellow portion of said image, wherein one of said gelatin-relief-image-containing matrices corresponds to the red portion of said image, and wherein one of said gelatin-relief-image-containing matrices corresponds to the blue portion of said image, and wherein a yellow dye is applied to said gelatin-relief-image-containing matrix corresponding to the yellow portion of said image, wherein a red dye is applied to said gelatin-relief-image-containing matrix corresponding to the red portion of said image, and wherein a blue dye is applied to said gelatin-relief-image-containing matrix corresponding to the blue portion of said image.

45 16. A method for forming a color image as claimed in claim 1, wherein said rehalogenating is repeated.

### References Cited

#### UNITED STATES PATENTS

|           |         |              |       |       |
|-----------|---------|--------------|-------|-------|
| 1,923,764 | 8/1933  | Troland      | ----- | 96—36 |
| 2,244,589 | 6/1941  | Yankel       | ----- | 96—12 |
| 2,607,684 | 8/1952  | Nowak et al. | ----- | 96—36 |
| 2,814,565 | 11/1957 | Long         | ----- | 96—12 |

70 NORMAN G. TORCHIN, Primary Examiner

A. T. SURO PICO, Assistant Examiner

U.S. Cl. X.R.